

## UNITED STATES PATENT OFFICE

1,981,522

## DISPERSION OF MINERAL MATTER

Oscar Frederick Neitzke, Belmont, Mass.

No Drawing. Application March 18, 1932,  
Serial No. 599,850

2 Claims. (Cl. 134—1)

This invention relates to the production of dispersions of thermo-plastic hydrocarbon materials, such as petroleum asphalt, mineral asphalt and the like, in an aqueous medium.

5 The main purpose of the invention relates to the production of dispersions of asphaltic material in an aqueous medium, which dispersion will be of relative high stability and which may be diluted sufficiently with water to have high penetration qualities, e. g., when applied in penetration type of road work.

10 It is of importance in emulsions of the type disclosed that the saponifiable material employed can be readily obtained in quantity and at a fair price in this country and that the material will not unduly detract from the quality of the asphalt after the emulsion has been applied.

15 It has been found that vegetable pitches, such as stearin pitch, which is a fatty acid pitch constituting the still residuum resulting from the distillation and purification of vegetable oils, such as cottonseed oil, can be used to furnish the protective colloid or stabilizer in emulsions 20 of mineral asphalts and pitches. This residuum is available at cottonseed oil refineries, for example, substantially as a waste product, since it has only limited applications commercially, due to its relatively poor weathering qualities when used alone. As available on the market the preferred form has a dark pitch-like body having approximately the following characteristics,— 25 specific gravity of 1.01, melting point of 100° F. to 153° F. (Ball and Ring), an acid number 60, 30 and a low unsaponifiable content, some examples being as low as approximately 5% to 8%. This material, known as stearin pitch in commerce, is completely miscible in any proportion with mineral asphalts, e. g., those derived from 35 the distillation of crude petroleum.

40 In forming the emulsion, the asphalt and vegetable pitch are brought to a temperature sufficiently high to liquefy them and they are completely mixed as by being boiled with steam or by having air passed upwardly through the same to produce a homogeneous mixture of the mineral asphalt and vegetable pitch.

45 Since there is no tendency in the mixed materials to separate out on solidification, the mixed 50 materials may be permitted to return to a solid state thereafter and then reheated to a fluid state, at the time of the formation of the dispersions. The dispersion may, however, be formed 55 while the materials are heated, as soon as they

have been mixed, and without permitting them to cool.

The dispersion is formed by introducing the melt, comprising the asphalt and vegetable pitch, with agitation into a body of water containing a small quantity of caustic soda or other alkali capable of serving as a saponifying agent for the saponifiable content of the melt. The caustic soda in solution apparently reacts with such free fatty acid or fatty acid glycerides as are present in the stearin pitch to generate soaps in situ throughout the heat liquefied mixture, these soaps serving to stabilize the particles of bitumen reduced to small particle size by the agitation when the melt is introduced into the aqueous medium. In the present instance, in addition to the breaking up of the materials into microscopic particles in the aqueous medium by the agitation which accompanies mixing the particles, I believe there is also a leaching 60 out of the soluble soap produced in the mass with the resultant release of fine particles of released bitumen broken up by the leaching action. In any event I have found that the particle size of the resulting dispersion is very small. 65

70 While different vegetable pitches differ considerably in their characteristics, it has been found that usually there is about 15% to 40% or higher by weight of the material which is saponifiable and which may be converted into soap functioning to stabilize the dispersion. In 75 practice it is desirable to use as large a proportion of asphalt as possible in the procurement of a stable dispersion. This is true because of the fact that as a rule asphalts are far more stable 80 when subjected to weathering than the vegetable pitches and most other stabilizing agents. If 85 too small an amount of the vegetable pitch is used, there results a dispersion in which the particles tend to separate out and coalesce so 90 that the dispersion does not have the necessary 95 stability, for example, for storage or transportation thereof.

100 It has been found that about 2½% of stearin pitch based on the weight of the mineral asphalt dispersed affords a dispersion of relatively poor stability, even though the materials are thoroughly saponified. As the ratio of the stearin pitch is increased the stability of the dispersion is correspondingly increased up to a certain limit, 105 but the weathering qualities of the product are correspondingly decreased. It is accordingly preferable to use the quantity of stearin pitch necessary to produce the stability required for a particular use. It has been found that emul- 110

sions containing from 2½% to 10% by weight, based on the mineral asphalt, provides a sufficient range of stability in the final product for all usual purposes. The products formed within 5 this range have sufficiently satisfactory bonding and weathering qualities for most purposes and particularly for road building and maintenance work.

Within the above range an emulsion formed 10 with 5% stearin pitch, based on the quantity of mineral asphalt employed, affords a highly stable emulsion of excellent weather-proofing qualities and the finished product can be diluted with water to as low as 50% to 60% solids content 15 without any marked tendency to coalescence or settling out of the particles. An emulsion of this type can readily be mixed with road building materials, such as sand and crushed stone, and when applied to the roadway the asphalt is 20 found to have the bonding qualities required for this type of work.

The following is an example of the formation 25 and use of the emulsion for road building purposes. A mixture of 95 parts of mineral asphalt of approximately 100° F. melting point and 150-200 penetration value is melted and thoroughly mixed with 5 parts of vegetable pitch, the mixture being heated to approximately 300° F. The melt so prepared is then mixed with an equal 30 volume of ¼% to ½% alkali metal hydroxide or carbonate water solution heated to 120° F. to 130° F., forming an emulsion of 50% solids content with a temperature of approximately 195° F. The water content may be as low as 30% 35 of the final dispersion. The particles of an emulsion so formed are uniformly small, being approximately one ten-thousandths of an inch in diameter.

The emulsion disclosed herein is particularly 40 useful for penetration type of road work, wherein the materials are laid in place and the asphalt poured over, into and through the crushed stone and other materials. The emulsion has a prop-

erty of high penetration and yet it breaks quickly when applied, this latter feature making it especially adaptable for this particular type of road work.

The quantity of stearin pitch employed does 80 not detract materially from the bonding qualities of the asphalt when applied to the crushed stone and sand aggregate, the dispersion forming a continuous body of bonding asphalt filling the interstices between the stone and sand. The time in which the emulsion breaks necessarily 85 varies under different atmospheric and other conditions, but in general the emulsion disclosed herein will break within about two hours after it has been applied.

While the examples given have been relatively 90 specific as required by the statutes for a complete disclosure of the invention, it will be understood that they are intended as examples only, and that the invention is to be limited 95 only as set forth in the appended claims.

What I claim is:

1. The process of forming an aqueous dispersion of asphalt comprising intimately mixing therewith from 2% to 5% of stearin pitch having 100 a relatively high saponification value and thereafter dispersing said mixture, while heated, in a dilute aqueous solution of a non-stabilizing alkali, and forming through the reaction of said pitch and alkali reaction products constituting 105 the essential stabilizing elements of the dispersion.

2. A dispersion whose solids content consists of from 95% to 98% mineral asphalt and from 2% to 5% stearin pitch, of the nature of cotton 110 seed oil foots pitch, dispersed in an alkaline aqueous medium, the alkalinity of which is supplied by less than 1%, based on the water content, of a substantially non-stabilizing alkali of the nature of caustic soda, the dispersion being 115 stabilized essentially by the reaction products of said pitch and said alkali.

OSCAR FREDERICK NEITZKE.

45

190

50

125

55

130

60

135

65

140

70

145

75

150